

[54] INOCULATING ALLOY FOR CAST IRONS

[76] Inventors: Louis G. Septier, "Cite Jardin";  
Jean-Claude G. Percheron, "Pen  
Duick", Rue des Maranches, both  
of Chedde, France

[22] Filed: July 19, 1971

[21] Appl. No.: 164,031

## [30] Foreign Application Priority Data

July 23, 1970 France ..... 7027144

[52] U.S. Cl. .... 75/130 R, 75/134 S

[51] Int. Cl. .... C22c 31/00, C22c 37/10

[58] Field of Search ..... 75/58, 130, 130 R,  
75/134 S, 123 L

## [56] References Cited

## UNITED STATES PATENTS

|           |         |                     |           |
|-----------|---------|---------------------|-----------|
| 2,139,515 | 12/1938 | Norris .....        | 75/123 L  |
| 2,950,187 | 8/1960  | Ototani .....       | 75/134 S  |
| 3,256,087 | 6/1966  | Pfluger et al. .... | 75/134 S  |
| 3,323,899 | 6/1967  | Forgeng et al. .... | 75/0.5 BA |
| 3,364,015 | 1/1968  | Sump .....          | 75/134 S  |

|           |        |                       |         |
|-----------|--------|-----------------------|---------|
| 2,705,196 | 3/1955 | Wever et al. ....     | 75/58   |
| 3,301,663 | 1/1967 | Wicher et al. ....    | 75/58   |
| 3,304,174 | 2/1967 | Ototani .....         | 75/58 X |
| 3,575,695 | 4/1971 | Miyashita et al. .... | 75/58 X |

## OTHER PUBLICATIONS

Metals Hdbk, 8th Ed., Vol. 1, p. 392 & Vol. 5, P. 358,  
ASM, 1961.Primary Examiner—L. Dewayne Rutledge  
Attorney—McDougall, Hersh & Scott

## [57] ABSTRACT

The present invention relates to the sphere of alloys intended for improving cast iron, including the inoculation of grey or spheroidal cast irons with an alloy having the following composition:

|                                                     |           |
|-----------------------------------------------------|-----------|
| —silicon                                            | 55 to 85% |
| —carbon                                             | 0.2 to 1% |
| —calcium                                            | 2 to 5%   |
| —aluminum                                           | up to 2%  |
| —the remainder being iron with<br>usual impurities. |           |

4 Claims, No Drawings

## INOCULATING ALLOY FOR CAST IRONS

The present invention relates to alloys intended for improving cast iron.

The variation in mechanical characteristics, as a function of the chemical composition of a lamellar grey iron, is well known. The composition of the cast iron is generally expressed by its equivalent carbon and it is, for example, known that the tensile strength increases with decrease in carbon equivalent.

However, it is known that the reduction in equivalent carbon causes an increase in the tendency of the cast irons to solidify as a white structure. In addition, the use of cast irons having low equivalent carbon causes the presence of interdendritic graphite on the micro-structure leading to poor characteristics in use.

On the other hand, it is known that an introduction, before casting, of silicon, in the form of an alloy or composite, known as "inoculating agents," has a much more pronounced graphitizing effect than the silicon introduced in the same form into the charge of cast iron.

The use of such inoculants enables the precipitation of the white structure to be avoided and thus the use of cast irons of low equivalent carbon and high mechanical characteristics.

On the other hand, it is well known that the use of inoculating alloys is not limited to grey cast iron and that such alloys used on spheroidal graphite cast iron permit the improvement in such characteristics as:

lengthening of the time before disappearance of the previously introduced nodulizing effect,  
refining of the grain,  
improvement of the structure by elimination of carbides.

It is known that the ferro-silicons of different grades are among the inoculating alloys which are most frequently employed in the practice of inoculation.

The beneficial action of carbon, in the inoculation of cast irons, is also well known and its action, as compared with that of silicon, is indicated in Table I.

TABLE I  
COMPARISON OF THE ACTION OF Si and C IN  
THE INOCULATION OF FOUNDRY IRONS

|    | Effect on the depth of temper | Effect on the graphitic structure | Effect on the structure of the matrix | Effect on the hardness of the matrix |
|----|-------------------------------|-----------------------------------|---------------------------------------|--------------------------------------|
| Si | reduction                     | enlargement                       | ferritization                         | softening                            |
| C  | reduction                     | refining                          | ferritization                         | softening                            |

Table I shows that the carbon acts in the same manner as the silicon as regards the depth of temper, the structure and the hardness of the matrix, and that it is able to counter-balance the effect of enlargement of the graphitic structure produced by the silicon.

It is well known that the ferro-silicons which are rich in silicon, even if they are manufactured in carburizing medium, contain little carbon. This is the case with industrial ferro-silicons which are generally employed for inoculating cast irons, so that it is not usually possible to take advantage of the beneficial action of the carbon for the inoculation. It has been proposed to make use of mixtures of ferrosilicon and graphite, but the use of this latter substance is not recommended when spheroidi-

dal graphite iron is prepared. In addition, such mixtures do not permit a regular distribution of the additives to be obtained which is as fine as that which can be obtained by the use of homogeneous alloys.

It is moreover known that calcium added to the ferro-silicon exerts a reinforcing effect on the inoculation, similar to that of carbon.

The object of the invention is an inoculating alloy of a novel Fe-Si-Ca-C type, which is more effective than ferro-silicons to which carbon or calcium has been added.

It is an unexpectedly established fact that the effects of the carbon and calcium, introduced into the ferro-silicon, are mutually reinforced, so that the gain obtained is better than the sum of the gains produced by the carbon and the calcium, when added individually.

The alloy of this invention contains 55 to 85 percent of silicon, 0.2 to 1 percent of carbon, 2 to 5 percent of calcium and up to 2 percent of aluminum, the remainder being iron plus its usual impurities which originate mainly from the initial materials. Commercial ferro-silicons are known which contain 1.3 to 1.5 percent of Al, 0 to 0.03 percent of Ti, 0 to 0.20 percent of Mn, 0 to 0.10 percent of Ni, 0 to 0.02 percent of Cr, 0 to 0.003 percent of S, 0 to 0.003 percent of P, 0 to 0.002 percent of Cu. Preferably, the alloy contains 70 to 80 percent of silicon, 0.3 to 0.7 percent of carbon, 2.0 to 4.0 percent of calcium, less than 1.5 percent of aluminum, while the remainder is iron. This alloy can be introduced into the cast iron by using the different procedures employed for the inoculation and peculiar to the foundry art.

Such an alloy can particularly be obtained by a process which consists in adding the carbon to a liquid alloy containing Si and Ca, by the addition of cast iron.

The following examples are given by way of illustration, and not by way of limitation, of the practice of this invention:

## Example 1

Into a synthesis induction furnace are introduced 12 kg of an SiCa alloy ( $Ca = 31.8$  percent) and 100 kg of industrial silicon ( $Si = 97.7$  percent). When the metal is liquid, 20 kg of small pieces of a hypereutectic cast iron titrating 5.6 percent of carbon are added. When the iron is dissolved, it is quickly poured. The product which is obtained contains:

Si = 78.7%  
C = 0.69%  
Ca = 2.81%  
Al = 1.10%

## Example 2

Into a ladle containing 198 kg of an industrial alloy in the liquid state and having the composition of:  $Si = 88.1$  percent,  $Ca = 4.83$  percent,  $Al = 1.3$  percent, iron and impurities being the balance for 100 percent, there are added, as in Example 1, 40 kg of a cast iron having 4.12 percent carbon.

When the iron is dissolved, it is quickly poured. The product which is obtained contains:

Si = 72.7%  
Ca = 3.62%  
C = 0.63 %  
Al = 1.04%

## Example 3

In a ladle containing 607 kg of an industrial alloy in the liquid state and having the composition of: Si = 90.1 percent, Ca = 2.8 percent, Al = 1.22 percent, the balance being iron and impurities, there are dissolved, as before, 120 kg of a cast iron containing 3.14 percent C and 2.3 percent Si. When the iron is dissolved in the starting alloy, it is quickly poured. The product which is obtained contains:

Si = 73.8%  
C = 0.47%  
Ca = 2.11%  
Al = 0.98%

## Example 4

Inoculation tests are carried out on an identical grey cast iron with the following products prepared according to the prior art and in accordance with the practice of this invention:

## Test I

For reference purposes, there is used a 75% ferrosilicon of the composition:

Si % = 75.7  
Ca % = 0.19  
C % = 0.05  
Al % = 1.10

with the balance being iron and impurities.

## Test II

There is used an alloy (not in accordance with the invention) which is rich in carbon and of the composition:

Si % = 74.2  
Ca % = 0.09  
C % = 0.31  
Al % = 1.11

with the balance being iron and impurities.

This alloy is obtained by synthesis from 98 percent silicon and cast iron with its supply of carbon.

## Test II A

There is used a mixture (not in accordance with the invention), which is rich in carbon and comprises:

75 percent Fe-Si (grain size 0.5 to 2 mm) ... 90 percent by weight

Graphite in grain form ..... 10 percent by weight

The 75 percent Fe-Si is the same as that of Test I.

## Test II B

There is used a mixture (not in accordance with the invention), which is rich in carbon and comprises:

75 percent Fe-Si (grain size 0.5 to 2 mm) ... 99.7 percent by weight

50

Graphite in grain form ..... 0.3 percent by weight

The 75 percent Fe-Si is the same as that of Tests I and II A.

## Test III

There is used an alloy (not in accordance with the invention) which is enriched in calcium and has the composition:

10 Si % = 75.4  
C % = 0.05  
Ca % = 3.58  
Al % = 1.09

with the balance to 100 percent being iron and impurities.

15 This alloy is elaborated by synthesis from: Si having a purity of 98 percent by weight Si-Ca containing 30 percent by weight Ca and iron.

## Test IV

There is used the alloy according to the invention as described in Example 2, the composition of which is repeated here:

Si % = 72.7  
25 Ca % = 3.62  
C % = 0.63  
Al % = 1.04

the balance to 100% being iron and impurities.

30 At 1450  $\pm$  10° C, a grey iron of mechanical type and having the following composition:

C % = 3.45  
Si % = 1.90  
Mn % = 0.54

35 P % = 0.1  
is inoculated under the same conditions in the runner as it is being poured.

For the entire series of inoculations, there are used under the same conditions the products I, II, II A, II B, III, IV, in a quantity such that the proportions of inoculating ferrous alloy represents 0.3 percent of the weight of the cast iron (i.e., an addition of 0.225 percent of silicon on the basis Si = 75 percent).

40 Each of the inoculation treatments is carried out in a ladle containing 40  $\pm$  2 kg of cast iron, and the additions, for the different alloys are:

| Inoculating products | Weight of inoculant added for 40 kg of cast iron (kg) |
|----------------------|-------------------------------------------------------|
| I                    | 0.120                                                 |
| II                   | 0.120                                                 |
| II A                 | 0.134                                                 |
| II B                 | 0.120                                                 |
| III                  | 0.120                                                 |
| IV                   | 0.120                                                 |

45 The comparison results obtained with the six products are set out in the following table:

TABLE II

| Inoculant                          | Number of eutectic cells per cm. <sup>2</sup> |           | Tempering depth, mm. (+) |           | Tensile strength |           | Brinell hardness |           |
|------------------------------------|-----------------------------------------------|-----------|--------------------------|-----------|------------------|-----------|------------------|-----------|
|                                    | Result                                        | Variation | Result                   | Variation | Result           | Variation | Result           | Variation |
| I (Fe-Si comparison)               | 164                                           | -----     | 12                       | -----     | 29.1             | -----     | 215              | -----     |
| II (Fe-Si-C)                       | 174                                           | +10       | 9.1                      | -2.9      | 28.6             | -0.5      | 209              | -6        |
| II A (Fe-Si plus 10% graphite)     | 210                                           | +46       | 9.8                      | -2.2      | 27.4             | -1.7      | 202              | -13       |
| II B (Fe-Si plus 0.3% graphite)    | 172                                           | +8        | 12.1                     | +0.1      | 28.7             | -0.4      | 217              | +2        |
| III (Fe-Si-Ca)                     | 196                                           | +32       | 8                        | -4        | 28.3             | -0.8      | 208              | -7        |
| IV (Fe-Si-Ca-C)                    | 241                                           | +77       | 4.8                      | -7.2      | 32.6             | +3.5      | 196              | -19       |
| Reminder: cast iron not inoculated | 83                                            | -----     | 18                       | -----     | 26.8             | -----     | 221              | -----     |

(+) On tempering test bar of "international" type.

It will be seen that test IV, representing the practice of this invention, gives the best results.

It will be understood that changes may be made in the details of formulation and application conditions,

TABLE III.—RESULTS OF INOCULATION ON SPHEROIDAL GRAPHITE CAST IRON

| Inoculating product                        | Appearance of the graphite | Mechanical characteristics (+1) |      |            | Structure on thin elements of 5 mm., percent |         | Analysis on elements, percent |      |             |
|--------------------------------------------|----------------------------|---------------------------------|------|------------|----------------------------------------------|---------|-------------------------------|------|-------------|
|                                            |                            | E.L.                            | R    | E, percent | Carbides                                     | Ferrite | C                             | Si   | Mg          |
| I, ferrosilicon low C and low Ca.....      | Spheroidal.....            | 36.1                            | 50.2 | 14.6       | 45                                           | 45      | 3.6                           | 2.69 | 0.042/0.044 |
| III, ferrosilicon low C and with Ca.....   | do.....                    | 31.5                            | 51.0 | 17.5       | 35                                           | 65      | 3.6                           | 2.71 | 0.042/0.044 |
| IV, Fe-Si-Ca-C according to invention..... | do.....                    | 31.9                            | 50.5 | 22.2       | <5                                           | 65      | 3.6                           | 2.67 | 0.042/0.044 |

NOTE.—Characteristics in respect of a bar machined from a solid piece:  
(+1) E.L.=elastic limit (kg./mm.<sup>2</sup>).  
R=tensile strength (kg./mm.<sup>2</sup>).  
E, percent=elongation percent.

The variation is different from that which it would have been possible to allow for when the effects of the carbon and calcium are added separately. In particular, the carbon and the calcium by themselves lead to a reduction in the tensile strength, whereas their presence together in the alloy results in an improvement in this characteristic.

#### Example 5

The products of tests I, II and IV of Example 4 are used this time for inoculating, for comparison purposes, a spheroidal graphite cast iron containing C = 3.9 percent and Si = 1.3 percent. It is known that the introduction of graphite, as in the tests IIA and IIB of the preceding example, is not recommended with this type of cast iron. After nodulization treatment with a magnesium alloy, the spheroidal graphite iron is inoculated, for comparison purposes, with the three products I, II and IV, all three being used in the amount of 0.75%:

inoculation temperature:  $1460 \pm 5^\circ \text{C}$

pouring temperature of the elements:  $1420 \pm 5^\circ \text{C}$

The compared results are set out in Table III.

The data confirms that there is a considerable gain as regards the elongation and a very substantial decrease in the percentage of carbides in the cast iron treated by the alloy according to the invention.

without departing from the spirit of the invention, especially as defined in the following claims.

We claim:

1. An alloy based on iron and silicon consisting essentially of  
20 55 to 85 percent by weight silicon  
0.2 to 1 percent by weight carbon  
2 to 5 percent by weight calcium  
less than 2 percent aluminum, the remainder being iron plus impurities.
2. An alloy as claimed in claim 1 in which the silicon is present in an amount within the range of 70 and 80 percent, the carbon is present in an amount within the range of 0.3 and 0.7 percent, the calcium is present in an amount within the range of 2 and 4 percent and the aluminum is below 1.5 percent by weight.
3. The process for the preparation of the alloy of claim 1 comprising adding cast iron to a liquid bath containing silicon and calcium.
4. In the metallurgy of grey and spheroidal graphite cast irons, the step of inoculating the cast iron with an alloy of claim 1.

\* \* \* \* \*

45

50

55

60

65